

## UNITED STATES PATENT OFFICE

GEORGE D. KNIGHT, OF REDWOOD CITY, CALIFORNIA, ASSIGNOR TO EMORY WINSHIP,  
OF SAN FRANCISCO, CALIFORNIA

## PRINTING INK BASE

No Drawing. Application filed April 16, 1924, Serial No. 706,881. Renewed June 30, 1927.

The invention relates to a printing ink and particularly to the base, vehicle or carrier to which the pigment is added to produce the finished ink.

5 An object of the invention is to produce an intaglio or engraving ink.

Another object of the invention is to produce a non-inflammable intaglio ink.

Another object of the invention is to produce an intaglio ink which will redissolve in the etching of the printing cylinder when the rotogravure press is started after a temporary shut down.

Another object of the invention is to provide an ink in which no stratification occurs and in which there is no sedimentation of the pigment.

Another object of the invention is to provide an intaglio ink which resists removal 20 by water after printing.

A further object of the invention is to provide a satisfactory and inexpensive intaglio ink and a process of making the same.

The invention possesses other advantageous features, some of which, with the foregoing, will be set forth at length in the following description, where I shall outline in full the preferred form of the ink of my invention and the method of making the 30 same.

The ink base of my invention consists principally of a colloidal solution of gelatin and casein. The gelatin is preferably animal glue and the casein may be derived from 35 any suitable source. While I have made successful rotogravure ink from a colloidal solution of glue, casein and water, plus a suitable casein solvent such as ammonia, I find that better results are obtained by employing skim milk as the source of casein.

Besides containing sufficient casein, the skim milk contains other ingredients, such as sugar of milk, albumen, and mineral salts, which apparently have a beneficial effect upon the 45 resulting product. Further, the casein contained in milk is cheaper than separated casein so that by employing skim milk, I not only produce a better product, but a cheaper product. Skim milk contains approximately ninety percent water, three per-

cent casein, and five percent milk sugar, seven tenths percent albumin and two tenths percent fat. While I prefer to use skim milk as the source of the casein, it is to be understood that I do not limit myself to the use 55 of skim milk, for this purpose, since separated casein may be used.

If the ink, or the ink base is to be stored for any considerable length of time before being used, I add a preservative to the solution to prevent the decomposition of the glue and such preservative is preferably an oxidizing agent, such as an alkali bichromate. I have employed potassium bichromate successfully. In the event that the odor of the 60 solution is offensive, the odor may be masked by adding a strong smelling oil, preferably a pungent oil, such as citronella oil, and this oil acts also as a preservative.

I find that by adding a vegetable oil to the 70 mixture, the viscosity of the emulsion is increased and the ink pulls more readily from the intaglio cylinder or plate in the printing operation. By adding the vegetable oil, the ink base is given a greater affinity for paper 75 than for the metallic printing cylinder or plate. I have found that linseed oil satisfied these requirements satisfactorily. In the event that the ink base is too stiff, a small percentage of a hydrocarbon thinner may be 80 added which dilutes, without destroying the emulsion.

When separated casein is employed it is mixed with a suitable solvent, such as an aqueous solution of ammonia to produce a 85 solution of substantially the same proportions as occur in skim milk. When skim milk is employed the ingredients are mixed together in approximately the following proportions by weight:

|                      |            |
|----------------------|------------|
| Skim milk            | 70% to 80% |
| Glue                 | 10% to 20% |
| Potassium bichromate | 2% to 4%   |
| Vegetable oil        | 3% to 4½%  |
| Citronella oil       | 1%         |
| Hydrocarbon thinner  | 2%         |

I have obtained very satisfactory results from a mixture of 75% skim milk and from 14% to 16% of glue and the other ingredi- 100

ents as given above. When vegetable oil is not used the percentage of the citronella oil should be increased to approximately 4%. Any suitable oxidizing agent may be employed and while I have used potassium bichromate, other metallic bichromates such as sodium and ammonium may be used with substantially equal effects. When separated casein is used the percentage of the bichromate is increased.

10 In making the ink base from skim milk the glue is first soaked in cold skim milk and the mixture is then heated to a temperature below the boiling point. The mixture is then introduced into a closed container, or the container within which it is mixed is closed and the mixture is subjected to heat to produce a pressure preferably from fifty to sixty pounds to the square inch within the container. The mixture is therefore subjected to a temperature of from 140° C. to 150° C. and the pressure and temperature are maintained for from one to three hours to insure the proper results. I have found that if the mixture is not boiled under pressure that it will gelatinize on cooling. After the mixture has been heated in the closed container for the proper amount of time it is permitted to cool in the closed vessel, while under pressure, and, by following this method the cooled material remains in liquid form. After being cooled, the liquid is filtered to remove lumps.

15 I have found that it is desirable to add the bichromate and the linseed oil to the mixture while it is hot, that is at approximately 80° C., and also to add the pigment while the mixture is at this temperature to obtain thorough dissemination of the pigment and to prevent settlement thereof, which has a tendency to occur if the pigment is added to the mixture after it has cooled. I have made successful ink by mixing from 90 to 110 parts by weight of pigment with 100 parts 20 by weight of the base or vehicle so that the finished ink contains from 45% to 55% of pigment. The pigment used was a mixture of manganese oxides, but oxides of other metals may be added, depending upon the color desired.

25 The bichromate or other oxidizing agent added to the mixture helps to fix it and also assists in preventing the removal of the ink from the paper after printing. The citronella oil is preferably added to the mixture after it has cooled to substantially normal room temperature. By following this process I am enabled to produce a very effective and relatively cheap intaglio ink, which is 30 non-inflammable which is resistant to removal by water after it has been imprinted on paper and which readily pulls from the depressions in the metallic engraving or etching. The ink may be readily washed 35 from the metallic plate or cylinder, when the

press is shut down, with a borax solution. Due to the non-inflammable nature of the ink, the press may be run at high speed since there is no danger of ignition.

I claim:

1. An intaglio ink including casein dissolved in an aqueous solution of ammonia combined with another glue.
2. An intaglio ink including casein dissolved in an aqueous solution of ammonia combined with animal glue.
3. An intaglio ink including casein dissolved in an aqueous solution of ammonia, and animal glue and an oxidizing agent.
4. An intaglio ink including casein dissolved in an aqueous solution containing ammonia, animal glue and an alkali bichromate.
5. An intaglio ink including casein dissolved in an aqueous solution containing ammonia, animal glue, an oxidizing agent, 85 and a vegetable oil.
6. An intaglio ink including casein dissolved in an aqueous solution containing ammonia, another glue, an oxidizing agent, a deodorant and a vegetable oil.
7. An intaglio ink including casein dissolved in an aqueous solution containing ammonia, another glue, and an alkali bichromate.

90 In testimony whereof, I have hereunto set my hand.

GEORGE D. KNIGHT.

100

105

110

115

120

125

130